

## UNITED STATES PATENT OFFICE

2,500,140

## SENSITIVE PHOTOGRAPHIC MATERIALS

Eric F. Teal and Edward P. Davey, Wealdstone, England, assignors to Eastman Kodak Company, Rochester, N. Y., a corporation of New Jersey

No Drawing. Application March 6, 1947, Serial No. 732,934. In Great Britain April 1, 1946

5 Claims. (Cl. 95—7)

1

This invention relates to sensitive photographic materials, and to sensitive silver halide developing-out emulsions, as contrasted with printing-out emulsions.

Developing-out emulsions can to-day be broadly divided into two classes, namely (1) those which give a strong negative image from mere development, that is to say, upon development the silver salt darkens most in those places where the most light fell during the image-wise exposure, and (2) those which give a strong positive image upon mere development, that is to say, upon development the silver salt darkens most in those places where the least light fell during the image-wise exposure.

The present invention is directed to the manufacture of emulsions of the latter class, which are known as direct positive emulsions. Such emulsions may be coated on films, plates, papers or tracing cloth or the like.

Emulsions of both classes (1) and (2) are made with similar ingredients which are usually compounded by much the same technique, except that for class (2), the emulsion is given an additional treatment. The reason for this is that nearly all developing-out emulsions of class (1) will tend to give a positive upon development if the image-wise exposure is long enough. The phenomenon has been known for a very long time and is called solarisation. The emulsions which are specially treated so as to fall into class (2), give a very much better positive and with little image-wise exposure.

Various methods of making direct positive emulsions are known, for instance, by merely pre-fogging an emulsion of class (1). Another method is to cause a chemical fogging during ripening. Another method is to incorporate in a finished emulsion about 1½ to 4 times the amount of a non-acid optical sensitizing dye required to give optimum sensitizing together with a photographic developing agent.

The problem to which most of the prior suggestions have been directed is to make a direct positive emulsion which requires relatively little image-wise exposure and upon development gives an image which is of good contrast with deep blacks and clean whites, but all known methods still leave much to be desired in these directions. The present invention enables improved results of this kind to be obtained.

In the present invention we employ reducing agents containing elements selected from groups IV, V and VI of the periodic table.

The present invention is based on the discovery

2

that greatly improved results of the kind indicated, can be achieved if in the manufacture of the emulsion there is present during the formation of the sensitive silver salt one or more of the following reducing agents, arsenites, stannites, phosphites, metaphosphites, hypophosphites, antimonites, hyposulphites and germanites. Alkali or ammonium salts are especially advantageous. These compounds reduce an ammoniacal solution of silver nitrate to silver, at least when the solution is warmed.

The emulsion may comprise silver bromo-iodide which is formed by adding a solution of silver nitrate to a solution of a soluble bromide and 15 a soluble iodide, in which case, the said reducing agent may be incorporated in the last mentioned solution.

Emulsions which have been ripened by treatment with ammonia are preferred, although non-20 ammoniacal emulsions will give a fair result. We preferably employ silver bromo-iodide emulsions containing up to 20% of silver iodide based on the total weight of silver bromide and iodide, but emulsions in which the only silver halide is silver 25 bromide can be used. Digestion of the emulsion (i. e. after washing) may be desirable in some cases. However, the emulsion may be coated if desired immediately after the ripening treatment (i. e. without washing).

30 In the examples below, the quantities in brackets give a rough idea of the amount usually found to give useful results in an amount of emulsion containing 100 grams of Ag.

35 Phosphites (e. g. metaphosphites and hypophosphites) give good speeds and very clean whites, for example,

Sodium metaphosphites,  $Na_3PO_2$  (2.36 grams)  
Sodium phosphites,  $Na_2HPO_3 \cdot 5H_2O$  (0.8 gram)  
Sodium hypophosphite,  $NaH_2PO_3 \cdot H_2O$  (1.6 40 grams).

Arsenites give good speeds and very clean whites, for example, commercial sodium arsenite (probably sodium metarsenite),  $NaAsO_2$  (3.1 45 grams).

Antimonites give good speeds and very clean whites, for example, sodium antimonite,  $NaSbO_3$  (1.6 grams).

50 Stannites give good results but have some tendency to cause staining, for example, sodium stannite,  $NaHSnO_3$  (0.008 gram).

Hyposulphites give very good results with clean whites in some cases, for example, sodium hyposulphite,  $Na_2S_2O_4 \cdot 2H_2O$  (0.016 gram). Sulphites have insufficient reducing power.

The above-mentioned antimonite was prepared specially by dissolving antimonous oxide in caustic soda. The stannite was prepared by adding caustic soda to stannous chloride solution ( $\text{SnCl}_2$ ), until the precipitate first formed was redissolved and using the solution so obtained.

If desired, the emulsion so made may also be chemically fogged or light fogged. Almost any known chemical fogging agent can be used but some cause dirty whites: the chemical fogging agent is preferably added before the end of the ripening step. Good results have been obtained using hydrazine formaldehyde, hydroxylamine or excess of silver nitrate. Mere extra digestion of the emulsion or extra digestion with sulphur sensitizers such as sodium thiosulphate can be used for this purpose.

We prefer to employ for the emulsion an ammoniacal type, for example:

*Solution A*

|                   |       |       |
|-------------------|-------|-------|
| Potassium bromide | grams | 132   |
| Potassium iodide  | do    | 11.5  |
| Gelatin           | do    | 60    |
| Reducing agent    | x     |       |
| Water             | cc    | 2,500 |

The reducing agent may be any one of the following, the quantity  $x$  being as indicated.

|                     |       |       |
|---------------------|-------|-------|
| Sodium arsenite     | grams | 3.5   |
| Sodium phosphite    | do    | 1.0   |
| Sodium hyposulphite | do    | 0.2   |
| Sodium stannite     | do    | 0.007 |

*Solution B*

|                |       |     |
|----------------|-------|-----|
| Silver nitrate | grams | 195 |
| Water to       | cc    | 400 |

To solution B at room temperature add slowly with stirring in the usual way, sufficient ammonia solution (0.880 sp. gr.) until the precipitate first formed is just redissolved and raise the temperature of the mixture to 65° C. Now add solution B to solution A at 65° C. taking a few minutes to effect this. Ripen the emulsion for 30 minutes at 65° C. Then add 200 grams of gelatin. Then ripen a further 15 minutes at 65° C. Then allow the emulsion to cool and set and wash in the usual manner, until the emulsion has a pH of 7.2. Melt the emulsion and add 50 ccs. of 20% solution of potassium bromide and make up to 3½ litres with water. The autopositive emulsion so made may now be coated and will give a positive image providing the exposure is sufficient. If it is found that the maximum density obtained in such positive image is insufficient, then instead of coating after washing, digest the emulsion for about ½ hour at 65° C. and then coat. Emulsions so made will give negative images on low exposures: the production of such negative images can be avoided by fogging the emulsion, for instance, the emulsion can be fogged chemically by adding say 0.05 to 0.2 gram of hydrazine hydrochloride or 3.0 ccs. of 20% formaldehyde to the emulsion immediately after solution B has been added to solution A.

The emulsions made according to the present invention, may be sensitized with sensitizing dyes especially mere-cyanines and cyanines and in this case the amount of dye may be advantageously greater than the optimum quantity of dye relative to the usual amounts used for sensitizing purposes, as described in United States Patent No. 2,184,013, it being not essential to add a developing agent as therein given.

If desired a developing agent such as hydroquinone can be incorporated in the emulsion so

that after exposure of the emulsion it can be developed merely by immersion in an alkaline solution. By using an unhardened emulsion, alkaline hydroquinone development or other tanning developer will tan the emulsion imagewise, in which case the untanned portions can be washed off immediately after development or at a later stage.

A typical developer which may be used for developing emulsions made according to the present invention is as follows:

|                           |       |      |
|---------------------------|-------|------|
| Elon                      | grams | 2.2  |
| Sodium sulphite (cryst.)  | do    | 144  |
| (or anhydrous)            | do    | (72) |
| 15 Hydroquinone           | do    | 8.8  |
| Sodium carbonate (cryst.) | do    | 130  |
| (or anhydrous)            | do    | (48) |
| Potassium bromide         | do    | 4    |
| (or 10% solution)         | cc    | (40) |
| 20 Water to make          | cc    | 1000 |

What we claim as our invention and desire to be secured by Letters Patent of the United States is:

25 1. The method of making a direct positive developing out silver salt emulsion which comprises forming the sensitive silver salt in the presence of an amount of a reducing agent of the class consisting of about 3.1 grams of an arsenite, about 0.008 gram of a stannite, from 0.8 to 2.36 grams of a phosphite, about 1.6 grams of an antimonite and about 0.016 gram of a hyposulphite, each per 100 grams of silver in the emulsion.

2. The method of making a direct positive developing out emulsion according to claim 1 wherein the emulsion is of the ammoniacal type.

3. The method of making a direct positive developing out silver salt emulsion according to claim 1 wherein the emulsion is fogged during manufacture.

4. A direct positive silver halide emulsion containing an amount of reducing agent of the class consisting of about 3.1 grams of an arsenite, about 0.008 gram of a stannite, from 0.8 to 2.36 grams of a phosphite, about 1.6 grams of an antimonite and about 0.016 gram of a hyposulphite, each per 100 grams of silver in the emulsion, said silver halide having been formed in said emulsion in the presence of at least one of said reducing agents.

5. A silver halide emulsion according to claim 4 and containing a developing agent.

ERIC F. TEAL.

EDWARD P. DAVEY.

**REFERENCES CITED**

The following references are of record in the file of this patent:

**UNITED STATES PATENTS**

|           |       |               |
|-----------|-------|---------------|
| Number    | Name  | Date          |
| 2,005,837 | Arens | June 25, 1935 |

**FOREIGN PATENTS**

|           |               |               |
|-----------|---------------|---------------|
| 65 Number | Country       | Date          |
| 462,730   | Great Britain | Mar. 15, 1937 |

**OTHER REFERENCES**

"British Journal of Photography," vol. 70, 70 November 23, 1923, pages 717-720. (Copy in Scientific Library.)

"The Photographic Journal," Great Britain, August 1924, pages 363-369. (Copy in Scientific Library.)